

## UNITED STATES PATENT OFFICE

2,072,265

MANUFACTURE OR TREATMENT OF  
TEXTILE AND OTHER MATERIALS

Edgar Bertie Johnson and Robert Pierce Roberts,  
Spondon, near Derby, England, assignors to  
Celanese Corporation of America, a corpora-  
tion of Delaware

No Drawing. Application January 23, 1934, Serial  
No. 707,929. In Great Britain February 8,  
1933

13 Claims. (Cl. 18—54)

This invention relates to the manufacture or treatment of textile and other materials to modify their properties or appearance, and has particular reference to the treatment of filaments, threads, 5 yarns and the like of organic derivatives of cellulose and fabrics containing the same, in order to reduce or destroy their lustre.

According to the present invention, the lustre of textile and other materials made of or containing organic derivatives of cellulose, and especially filaments, threads, yarns and like materials and fabrics containing the same is reduced by subjecting such materials containing an oil, fat or the like and in a substantially dry condition, to the action of heat. The materials treated may be made of or may contain organic esters or ethers of cellulose, either simple or mixed or mixed ether-esters. Examples of cellulose esters are, cellulose formate, cellulose acetate and cellulose propionate, whilst cellulose ethers include methyl cellulose, ethyl cellulose and benzyl cellulose.

Vegetable oils are found to give very satisfactory results in the present connection, and especially oils of cocoanut and like origin. In particular, cocoanut oil itself has been found in practice to be eminently suitable in the present connection.

It is preferred to incorporate the oil, fat or the like into the textile material by making it one of the ingredients of the solution from which filaments are spun by a wet or dry spinning process. In a method of carrying this out which has been found particularly convenient in practice, and productive of very satisfactory results the oil, fat or the like is added to and well mixed with a cellulose derivative spinning solution which is then spun into an evaporative atmosphere; thus cocoanut oil may be added to an acetone solution of cellulose acetate. In the case of dry spinning the filaments emerging from the spinning apparatus are substantially free from moisture, but where a wet spinning process is involved, or where the filaments or yarn undergo a treatment involving the presence of moisture, or are moist for any other reason, such moisture should be driven off before the application of heat for delustering the materials in accordance with the present invention. This drying may conveniently be effected, for example, by passing the materials through a jacket or chamber warmed by steam or electrical means, or by directing warmed air upon them.

Other methods of incorporating the oil, fat or the like than by making it one of the ingredients

of the spinning solution may, however, be employed. Whatever method is adopted the oil, fat or the like may be incorporated as such or in the form of solutions or emulsions.

The application of heat to the treated material 5 in accordance with the invention may be made in various ways. Most conveniently, however, the materials are brought into contact with a heated surface, for example a hollow rod or roller internally heated by steam or electrical means. The 10 filaments or yarn containing the oil are passed over or around one or more of such rods or rollers, or between one or more pairs of hollow nipping rollers, either or both rollers of each pair being internally heated. This heat treatment is conveniently applied to the materials immediately or shortly after their formation, and in cases where the oil is incorporated in a spinning solution from which filaments are dry spun by extrusion into an evaporative atmosphere, the 15 substantially dry filaments emerging from the spinning apparatus may be passed around one or more heated rollers during their travel to a cap- 20 twisting or other filament-associating device.

The temperature to which the materials are 25 subjected during the heat treatment is naturally limited by the temperature at which they melt. When a textile material, e. g. a filament, yarn or fabric, is treated, temperatures of about 210° C. should not be exceeded if stiffening is to be avoided 30 unless the material contains substances adapted to raise its sticking point. Usually temperatures of about 160 to 210° C. and particularly 180 to 200° C. are efficacious.

It has been found that a heat treatment 35 according to the invention may not be accompanied by an immediate loss of lustre in the materials, but that a gradual and progressive diminution in lustre may be initiated by such treatment. For example, it has been observed, 40 on applying heat to filaments of cellulose acetate containing about 10% of cocoanut oil, that no appreciable delustering is apparent immediately after such treatment, but that the materials gradually lose lustre, on standing over a period 45 of a day or more.

The actual quantity of oil applied to the materials may be, for example, 5 to 15% by weight relative to the cellulose derivative present, quantities of about 10% being particularly ad- 50 vantageous.

Whilst it has been found possible, by treating filaments, yarns and fabrics in accordance with the present invention, to reduce their lustre to such an extent that they present an entirely 55

dull matt appearance, it has also been discovered that the presence of moisture on the materials during the heating step reduces or nullifies the dulling effect of the heat. Further, it is even possible to renew the lustre, on materials which have been dulled in accordance with the present invention, by moistening the materials and re-heating them, and the invention extends to such subsidiary operations.

10 It will therefore be realized that the degree of delustering produced by the present process may be controlled not only by regulating the degree of heating of the materials, but also by regulating the amount of moisture present when 15 such heat is applied. Further, by varying the moisture present at different parts of filaments, yarns or fabrics, the degree of delustering produced will vary in such different parts, whereby 20 very pleasing differential-lustre effects may be obtained.

For example, moisture may be intermittently applied to travelling filaments or yarns, as by 25 a rotating moistening device having a discontinuous surface, or by moving the material into and out of contact with a moistening device by means of an oscillating guide or rotating cam. Alternatively, in the case of a fabric, moisture 30 may be applied to pre-selected areas thereof with the aid of a stencil. By applying heat to the materials so treated the lustre of the dry portions only thereof may be reduced, or, in cases where the entire material has already been uniformly delusted in accordance with the present 35 invention before such moistening, the moist parts thereof will regain their lustre. In either case differential-lustre effects are produced on the fabric or yarns so treated, or on fabric subsequently produced from such yarns.

The following example illustrates a convenient 40 method of carrying out the process of the invention, but it is to be understood that this example is given solely by way of illustration and is in no way limitative.

#### Example

45 Cocoanut oil is added to a 25% solution of cellulose acetate in a solvent mixture consisting of 95% acetone and 5% methyl alcohol in quantity equal to 10% on the weight of the cellulose 50 acetate and the product, after thorough mixing, is spun into an evaporative atmosphere.

The filaments leaving the spinning cabinet are fed, in their travel to a cap-twisting apparatus, first around a feed roller and then around a 55 roller heated internally to a temperature of about 195° C. By adjusting the speeds of the feed roller and heated roller any desired stretch may be applied to the filaments.

The yarn formed, after storage for a day, is 60 of matt appearance.

What we claim and desire to secure by Letters Patent is:—

1. Method of producing filaments, threads, 65 yarns, fabrics and other materials, comprising an organic derivative of cellulose, of low lustre, which comprises subjecting such materials, while containing an oleaginous substance and in a substantially dry condition, to the action of heat until a loss of lustre occurs at least after standing, the heat treatment being insufficient to 70 vaporize the oleaginous substance from the materials.

2. Method of producing filaments, threads, 75 yarns, fabrics and other materials of low lustre, which comprises extruding into a coagulating

medium a solution containing an organic derivative of cellulose and an oleaginous substance, and subjecting to the action of heat while in a substantially dry condition filaments so produced until a loss of lustre in the filaments occurs at least after standing, the heat treatment being insufficient to vaporize the oleaginous substance from the filaments. 5

3. Method of producing filaments, threads, 10 yarns, fabrics and other materials of low lustre, which comprises extruding into an evaporative atmosphere a solution containing an organic derivative of cellulose and a vegetable oil, and subjecting to the action of heat while in a substantially dry condition filaments so produced until 15 a loss of lustre in the filaments occurs at least after standing, the heat treatment being insufficient to vaporize the vegetable oil from the filaments.

4. Method of producing filaments, threads, 20 yarns, fabrics and other materials of low lustre, which comprises extruding into an evaporative atmosphere a solution containing an organic derivative of cellulose and 5 to 15% of cocoanut oil, and subjecting to the action of heat at temperatures of 160 to 210° C. while in a substantially dry condition filaments so produced until 25 a loss of lustre in the filaments occurs at least after standing, the heat treatment being insufficient to vaporize the cocoanut oil from the fil- 30 aments.

5. Method of producing filaments, threads, 25 yarns, fabrics and other materials, comprising cellulose acetate, of low lustre, which comprises subjecting such materials, while containing an 35 oleaginous substance and in a substantially dry condition, to the action of heat until a loss of lustre occurs at least after standing, the heat treatment being insufficient to vaporize the oleaginous substance from the materials. 40

6. Method of producing filaments, threads, 45 yarns, fabrics and other materials of low lustre, which comprises extruding into a coagulating medium a solution containing cellulose acetate and an oleaginous substance, and subjecting to 50 the action of heat while in a substantially dry condition filaments so produced until a loss of lustre in the filaments occurs at least after standing, the heat treatment being insufficient to vaporize the oleaginous substance from the filaments.

7. Method of producing filaments, threads, 55 yarns, fabrics and other materials of low lustre, which comprises extruding into an evaporative atmosphere a solution containing cellulose acetate and an oleaginous substance, and subjecting to the action of heat while in a substantially dry condition filaments so produced until a loss of lustre in the filaments occurs at least after standing, the heat treatment being insufficient to 60 vaporize the oleaginous substance from the filaments.

8. Method of producing filaments, threads, 65 yarns, fabrics and other materials of low lustre, which comprises extruding into an evaporative atmosphere a solution containing cellulose acetate and a vegetable oil, and subjecting to the action of heat while in substantially dry condition filaments so produced until a loss of lustre in the filaments occurs at least after standing, the heat treatment being insufficient to 70 vaporize the vegetable oil from the filaments.

9. Method of producing filaments, threads, 75 yarns, fabrics and other materials of low lustre, which comprises extruding into an evaporative

atmosphere a solution containing cellulose acetate and cocoanut oil, and subjecting to the action of heat while in a substantially dry condition filaments so produced until a loss of lustre in the filaments occurs at least after standing, the heat treatment being insufficient to vaporize the cocoanut oil from the filaments.

10. Method of producing filaments, threads, yarns, fabrics and other materials of low lustre, which comprises extruding into an evaporative atmosphere a solution containing cellulose acetate and 5 to 15% of cocoanut oil, and subjecting to the action of heat while in a substantially dry condition filaments so produced until a loss of lustre in the filaments occurs at least after standing, the heat treatment being insufficient to vaporize the cocoanut oil from the filaments.

11. Method of producing filaments, threads, yarns, fabrics and other materials of low lustre, which comprises extruding into an evaporative atmosphere a solution containing cellulose acetate and a vegetable oil, and subjecting to the action of heat at temperatures of 160 to 210° C., while in a substantially dry condition, filaments so produced until a loss of lustre in the filaments occurs at least after standing, the heat treatment being insufficient to vaporize the cocoanut oil from the filaments.

ment being insufficient to vaporize the vegetable oil from the filaments.

12. Method of producing filaments, threads, yarns, fabrics and other materials of low lustre, which comprises extruding into an evaporative atmosphere a solution containing cellulose acetate and cocoanut oil, and subjecting to the action of heat at temperatures of 160 to 210° C. while in a substantially dry condition, filaments so produced until a loss of lustre in the filaments occurs at least after standing, the heat treatment being insufficient to vaporize the cocoanut oil from the filaments.

13. Method of producing filaments, threads, yarns, fabrics and other materials of low lustre, which comprises extruding into an evaporative atmosphere a solution containing cellulose acetate and 5 to 15% of cocoanut oil, and subjecting to the action of heat at temperatures of 160 to 210° C., while in a substantially dry condition, filaments so produced until a loss of lustre in the filaments occurs at least after standing, the heat treatment being insufficient to vaporize the cocoanut oil from the filaments.

EDGAR BERTIE JOHNSON. 25  
ROBERT PIERCE ROBERTS.